

Patented Aug. 16, 1949

2,478,954

# UNITED STATES PATENT OFFICE

2,478,954

## METHOD OF TREATING PHOSPHATE COATED SURFACES

Bertha S. Tuttle, Newton, and Thaddeus Navoy,  
Jamaica Plain, Mass., assignors to J. N. Tuttle,  
Inc., Newton, Mass., a corporation of Massa-  
chusetts

No Drawing. Application April 27, 1944,  
Serial No. 533,062

16 Claims. (Cl. 148—6.1)

1

This invention relates to a method of treating phosphate-coated surfaces, such as are commonly applied to ferrous and ferrous alloy articles, to increase their corrosion resistance and if desired to impart a color thereto.

It has long been known that zinc, cadmium and ferrous surfaces may be rendered more or less corrosion resistant by treatment with phosphoric acid and/or phosphates of such metals as manganese, iron, zinc, copper and combinations thereof, with or without oxidizing agents or depolarizers, etc., typical procedures being disclosed in U. S. Patents No. 1,651,694 and No. 1,911,726, each of which embodies the use of a compound having the empirical formula  $M(H_2PO_4)_2$ , wherein M may be a metal from manganese to cadmium in the electromotive series. Since the essential ingredient embodied in such treatments is the phosphate radical, the processes are generally referred to as phosphate treatments, being commercially known as Parkerizing, Bonderizing, Granodizing, etc. It has also been found that the efficacy of the phosphate treatment may be enhanced and the character of the resultant phosphate coating varied by the use of salts of metals below iron in the electromotive series, and to this end minor amounts of salts of such elements as copper, silver, lead, tin, antimony, arsenic, etc., along with the principal ingredient, e. g.,  $M(H_2PO_4)_2$ , have been suggested. However, in all such modified procedures the essential or primary ingredient is the metal phosphate which provides at least the major portion of the corrosion resistant coating, the other ingredients being of secondary importance in that they either concomitantly form an additional phosphate complex along with the principal phosphate coating, or function apparently as an accelerator, catalyst or the like.

Such processes are generally unsatisfactory without supplementary treatments such as oiling, waxing, painting, etc., principally because they do not provide a high degree of corrosion resistance. A further deficiency in the phosphate treatment as commercially practiced is that it does not readily and satisfactorily permit fast coloring of the treated surface other than by the application of a coat of paint or lacquer, which inevitably results in objectionable dimensional changes.

The principal objects of the present invention are to provide a composition for and method of treating phosphate-coated surfaces so as greatly to increase their corrosion resistance; to provide a composition for and method of simultaneously

2

increasing the corrosion resistance of phosphate-coated articles and imparting thereto a desired coloration which can not be rubbed or washed off, which does not produce appreciable dimensional changes and which is relatively fast to light; and to provide a protective phosphate coating which is denser, more adherent, refined and smoother than the phosphate coatings heretofore produced, and which is resistant to heat and generally more attractive.

Further objects will be apparent from a consideration of the following description wherein we have disclosed several illustrative examples of what is now considered a preferred procedure embodying the use of typical compositions coming within the scope of the present invention.

We have found that articles having a phosphate coating such as produced by any of the well-known commercial procedures may be treated with an aqueous solution of a stannous salt which reacts with the phosphate coating to produce a highly resistant, smooth, dense coating consisting essentially of a tin-metal-phosphate complex, which has a corrosion resistance many times greater than that produced by any of the procedures heretofore used, as indicated by the standard salt spray test; and that if a compatible dye be incorporated in the stannous salt solution, the dye apparently becomes chemically combined with the tin-metal-phosphate complex and the resultant coating not only is given a coloration which is relatively fast to light and unaffected by water and solvents, but also is rendered more corrosion resistant than the tin-metal-phosphate coating without the dye. We have also found that by incorporating in the stannous salt solution certain stabilizers or inhibitors such as mannitol, gum arabic, dextrose and the like soluble carbohydrates, gelatine and similar hydrophilic colloids, the corrosion resistance of the resultant coating is likewise greatly increased.

In accordance with the present invention, the material to be treated, for example an article composed of iron, steel, a ferrous alloy, etc., is first subjected to any treatment capable of producing a phosphate coating, and to this end the article may be treated in accordance with any of the well known commercial procedures such, for example, as are disclosed in U. S. Patents Nos. 1,007,069, 1,651,694 and 1,911,726. The phosphate coating thus produced consists essentially of a relatively insoluble porous crystalline film-like structure formed on or integral with the surface of the treated article, and, without supplement-

tary treatment such as oiling, waxing, etc., has a corrosion resistance of the order of two to six hours, as determined by the standard salt spray test.

After having formed the phosphate coating base as above described, the article is next treated with an aqueous solution containing as its essential ingredient a soluble stannous salt at a temperature which may vary from room temperature to the boiling point of the solution and for a period which may vary from a few seconds to several minutes, depending upon the particular stannous salt used, the character of the basic phosphate coating, and the desired degree of corrosion resistance. The resultant coating is the reaction product of the stannous salt and the original phosphate coating and consists essentially of a tin-metal-phosphate complex which is not only smoother, more dense, fine-grained and scratch resistant than the phosphate coating base, but also many times more corrosion resistant. If it be desired to produce a greater corrosion resistance and/or coloring of the resultant coating, a dye soluble in and compatible with the stannous salt solution may be incorporated in the treating bath or solution, and in either case, if desired, a suitable stabilizer or inhibitor may also be added to the treating solution. The resultant coating consists essentially of a tin-metal-phosphate-dye complex which not only possesses increased corrosion resistance, as compared to the tin-metal-phosphate coating, but also an attractive coloration which is relatively fast to light and heat, and unaffected by water and solvents, and furthermore does not undergo an objectionable darkening when treated with oil and wax. After having completed the above treatment, with or without coloration, the article may then be rinsed off, dried, and, if desired, oiled or waxed in accordance with conventional practices.

The stannous salts suitable for use in our process are limited to those that are water soluble and relatively stable, and whose acidity may, if necessary, be adjusted so that the phosphate coating base is not stripped. Such salts comprise the stannous halides, stannous sulphate, stannous fluoborate, and certain organic stannous salts, such as the acetate, oxalate and tartrate. Practical considerations, however, indicate the use of the chloride, viz.,  $\text{SnCl}_2 \cdot 2\text{H}_2\text{O}$ , which has been found most satisfactory when used in concentrations varying from less than 1% to the saturation point of the salt, although preferred working limits are between 2% and 25%.

The dye or coloring agents suitable for use in our process include the synthetic organic dye-stuffs and certain animal and vegetable dyes which are compatible with an aqueous stannous salt solution having an acid pH. Recognized classifications of dyes, such as are found in the Colour Index (edited by F. M. Rowe and published under the auspices of the Society of Dyers and Colourists), offer little or no assistance in determining the particular types of dyes which are operative or suitable in our process. (In general dyes containing azo and nitro groups are inoperative, while the acid dyes of the triphenylmethane and xanthene types are operative.) However, the operability of any particular dye may readily be determined, and as a practical matter should be checked, by testing its compatibility with an aqueous 5% stannous chloride solution. If the dye causes the formation of a precipitate or becomes discolored it is incompatible.

Thus the dyes which are compatible are those which are soluble in an aqueous 5% stannous chloride solution without causing the formation of substantial precipitate or undergoing discoloration during a substantial period, e. g. one hour. Among the dyes which have been tested and found to be satisfactory are the following:

|    | Trade Name of Dye               | Identification or Colour Index No. |
|----|---------------------------------|------------------------------------|
|    | Anthraquinone Green G.....      | 1078                               |
|    | Alkali Fast Green.....          | 735                                |
|    | Safranine T (1).....            | 841                                |
|    | Rhodamine 6GDN (2).....         | 752                                |
| 15 | Alizarin Red S (3).....         | 1034                               |
|    | Wool Fast Blue.....             | 833                                |
|    | Acid Green L.....               | 666                                |
|    | Acid Green B.....               | 667                                |
|    | Wool Violet 4BN.....            | 668                                |
|    | Alizarine Blue GRL.....         | 1088                               |
|    | Alphasurine FG.....             | 671                                |
|    | Quinolene Yellow.....           | 801                                |
| 20 | Wool Green S.....               | 737                                |
|    | Alizarol Cyanine (3).....       | 722                                |
|    | Rhodamine B Extra (2).....      | 749                                |
|    | Brilliant Fuchsine (4).....     | 677                                |
|    | Brilliant Wool Blue FFR.....    |                                    |
|    |                                 | a triphenyl-methane acid dye.      |
|    | Phosphine GN (5).....           | 793                                |
|    | Induline.....                   | 861                                |
| 25 | Alizarol Blue Black (3).....    | 1085                               |
|    | Anthraquinone Blue B.....       | 1054                               |
|    | Anthraquinone Violet.....       | 1080                               |
|    | Alizarol Sapphire SE.....       | 1053                               |
|    | Brilliant Wool Blue GL (6)..... |                                    |
|    | Acid Magenta (5).....           | 692                                |
|    | Novazol Acid Blue GL.....       |                                    |
| 30 | Acid Red XG.....                | 745                                |
|    | Novazol Acid Blue SL.....       |                                    |
|    | Acid Red XB.....                | 748                                |
|    | Quinolene Yellow F.....         | 833                                |
|    | Erio Fast Fuchsine (4).....     | 749                                |
|    | Fast Acid Violet GRF.....       | 753                                |
|    | Anthraquinone Blue RXO.....     | 1076                               |
|    | Methylene Blue (5).....         | 922                                |

All dyes above listed, except those followed by a parenthetical numerical notation, are classified as acid dyes. The notations designate the following classifications:

- (1) Azine basic type
- (2) Phthalic anhydride type
- (3) Mordant acid type
- (4) Acid and basic type
- (5) Basic type
- (6) Unclassified

The amount or concentration of the dye will depend on the particular dye and the depth of coloration desired, but as a general rule from 50 0.1% to 10%, based on the weight of the treating solution, which is equivalent to a minimum of 0.4% of dye based on the weight of stannous salt within the above range, constitute practical working limits. However small quantities of other compatible dyes may be added for shading.

The use of a stabilizer or inhibitor may be desired, particularly where maximum corrosion resistance is of the utmost importance, and to this end the treating bath or solution may include 60 such stabilizers or inhibitors as mannitol, gum arabic, dextrose, sugar and the like carbohydrates, or gelatine and other types of hydrophilic colloids. However, it should be understood that the use of a stabilizer or inhibitor, although 65 sometimes advisable, is generally unnecessary, and where the use of a stabilizer is indicated, the amount to be used may, as a practical matter, vary between 10% and 40%, based on the weight of the stannous salt, depending upon the length of the period during which the treating solution or bath is to be used.

A procedure illustrative of the foregoing is as follows:

Example 1.—A stannous salt solution is first 75 prepared by dissolving 50 parts (by weight) of

commercial stannous chloride in 1000 parts of water, after which the solution is brought to boiling. Metallic tin may, if desired, be added to stabilize the bath, although satisfactory results may be secured without such addition. Steel, iron or other ferrous metal pieces, previously phosphate coated in conventional manner employing the Parkerizing Process, are then dipped in the stannous chloride for approximately one minute while at boiling temperature, after which the pieces are removed, rinsed and dried. A smooth, fine-grained, dense coating having a gray coloration is produced.

*Example 2.*—The procedure set forth in Example 1 was followed, except that 10 parts of Fast Acid Green B dye were incorporated in the stannous chloride solution with the result that a dark green coloration, fast to light and washing, was imparted to the coating.

*Example 3.*—The procedure set forth in Example 1 was followed, except that 10 parts of mannitol were added to the stannous chloride solution. The appearance of the coating was

Further tests on the dyed coatings (Examples 2 and 4 to 6) indicated that the coloration was fast to strong light, water and solvents.

In order to determine whether or not the incorporation of the dye in the stannous salt solution, as in Examples 2 and 4 to 6, produced results appreciably different from those obtained by treating phosphate-coated pieces, as in Example 1, and subsequently subjecting the pieces to a dip in a hot 1% dye solution, a series of tests were conducted in which (a) different dyes were incorporated in the stannous chloride solution following the procedure set forth in Example 2, and a second series of tests were conducted in which (b) the pieces were treated as in Example 1 and then dipped in a hot dye solution containing the same amount of dye as the corresponding test under (a). The following table shows the treatments and the results obtained, it being understood that the examples marked *a* follow the procedure of Example 2 and those marked *b* follow the procedure of Example 1 with a subsequent dye dip:

| Example | Dye                | Coloration            | Salt Spray Test         |
|---------|--------------------|-----------------------|-------------------------|
| 7a.     | Acid Green L.      | Medium Green          | Greater than 125 hours. |
| 7b.     | do                 | Very Light Green      | 40 hours maximum.       |
| 8a.     | Acid Green B.      | Dark Green            | Greater than 125 hours. |
| 8b.     | do                 | Light Green           | 50 hours maximum.       |
| 9a.     | Wool Violet 4BW    | Red-Violet            | 70 to 90 hours.         |
| 9b.     | do                 | Dark Uneven Staining  | 40 hours maximum.       |
| 10a.    | Alizarine Blue GRL | Very Light Blue       | 70 hours.               |
| 10b.    | do                 | Colorless             | 35 hours maximum.       |
| 11a.    | Alphasurine FG.    | Light Blue-Green      | 90 hours.               |
| 11b.    | do                 | Very Pale Bluish Tint | 40 hours.               |
| 12a.    | Quinolene Yellow   | Light Green-Yellow    | Greater than 70 hours.  |
| 12b.    | do                 | No coloration         | 35 hours maximum.       |
| 13a.    | Wool Green S.      | Dark Green-Blue       | Greater than 70 hours.  |
| 13b.    | do                 | Light Blue            | 50 hours maximum.       |
| 14a.    | Alizarol Cyanine   | Red-Violet            | Greater than 70 hours.  |
| 14b.    | do                 | Light Violet Tint     | 40 hours maximum.       |

substantially the same as that produced by Example 1.

*Example 4.*—The procedure set forth in Example 2 was followed using 10 parts of Wool Green S and 2 parts of sodium carbonate in place of the Fast Acid Green B. The resultant coating was similar to that produced by Example 1, except the coloration was a dark green-blue.

*Example 5.*—The same procedure as set forth in Example 2 was followed using 10 parts of Quinolene Yellow and the resultant coating had a light green-yellow coloration.

*Example 6.*—The same procedure set forth in Example 2 was followed using approximately 10 parts of a dye mixture which produced a coating having an olive drab coloration.

The pieces treated by each of the above procedures, without supplementary treatment, were then subjected to the standard salt spray test, along with the untreated phosphate-coated pieces, and the results are shown in the following table:

Table

| Treatment              | Initial Rusting | Substantial Rusting (50%+) |
|------------------------|-----------------|----------------------------|
| Plain Phosphate-coated | Hours           |                            |
| Example 1.             | 2 to 6          | 15 hours.                  |
| Example 2.             | 15 to 53        | 70 to 91 hours.            |
| Example 3.             | 82 to 104       | Greater than 104 hours.    |
| Example 4.             | 34 to 50        | 70 hours.                  |
| Example 5.             | 31 to 48        | 65 to 104 hours.           |
| Example 6.             | 53              | greater than 91 hours.     |
|                        | 65 to 82        | 104 hours.                 |

It will be observed that in each case there is not only a greater resistance to corrosion when the dye is incorporated in the stannous salt solution, but also the coloration produced on the coating is appreciably different, thus clearly indicating that the action of the dye when incorporated in the stannous salt solution is at least much more efficacious, i. e., not only imparting the desired coloration to the coating, but also greatly increasing its resistance to corrosion, than when the treated pieces are merely dipped into a dye solution.

Further tests confirming the foregoing were conducted using other types of dyes, including Anthraquinone G, Alkali Fast Green 2G, Safra-nine T, Rhodamine 6GDN, Alizarine Fast Blue, and Wool Fast Blue.

Examples representative of other stannous salt solutions as follows:

*Example 15.*—A stannous salt solution was first prepared by dissolving 50 parts (by weight) of stannous sulfate in 1000 parts of water, after which 13 parts of sodium carbonate were added. A piece of ferrous metal having a phosphate coating was then dipped into the treating solution for a period of ten minutes during which the solution was maintained at boiling temperature. A smooth, fine-grained, dense coating, comparable to that of Example 1, was produced. Salt spray tests showed an initial corrosion resistance of 15 hours as compared to 2-3 hours for the untreated phosphate coating, a corrosion resistance rating after 33 hours of 7, as compared to a rating of 3 for the untreated coating, and a

7 corrosion resistance of greater than 60 hours for the treated piece, as compared to 15 hours for the untreated piece.

*Example 16.*—A stannous sulfate solution was prepared as in Example 15, and 10 parts of Fast Acid Green B were added thereto. A piece of ferrous metal having a phosphate coating was then subjected to treatment as in Example 15, with the result that a dark green coloration, fast to light and washing, was produced. The coating showed an initial corrosion resistance of 33 hours and substantial rusting after more than 70 hours.

*Example 17.*—A stannous sulfate treating solution was prepared as in Example 16, except that 12.5 parts of sodium carbonate and 10 parts of Wool Green S were used. The phosphate coated metal was treated for ten minutes at boiling temperature with the result that a coating having a blue green coloration was produced. This coating showed an initial corrosion resistance of approximately 35 and substantial rusting after 70 hours.

*Example 18.*—A stannous salt solution was prepared by dissolving 50 parts of stannous fluoborate in 1000 parts of water, after which 10 parts of sodium carbonate was added. A phosphate coated piece of ferrous metal was then dipped into the solution maintained at boiling temperature for one minute. A coating comparable to that of Example 1 was produced, which had an initial corrosion resistance of 6 to 15 hours and substantial rusting after 50 hours.

*Example 19.*—A stannous fluoborate solution was prepared as in Example 18, and 10 parts of Fast Acid Green B were added to the solution. The test pieces were dipped for one minute in the solution while maintained at boiling temperature. A colored coating similar to that of Example 16 was produced, which coating had an initial corrosion resistance of approximately 25 hours with substantial rusting after more than 70 hours.

*Example 20.*—A stannous fluoborate solution was prepared as in Example 19, except that 10 parts of Wool Green S were added instead of the Fast Acid Green B. The test pieces were dipped in the treating solution for five minutes while maintained at boiling temperature. The resultant coating was comparable to that of Example 17, having a corrosion resistance better than that of Example 18, but less than that of Example 19.

All salt spray tests, herein referred to, were made on unoiled test pieces so that the efficacy of the various treatments could be determined more accurately. It is to be understood, however, that such supplementary treatments as oiling, waxing, etc., will substantially increase the corrosion resistance of both the untreated phosphate coated pieces and those treated in accordance with the present invention.

Experiments using organic stannous salts, viz., the acetate, oxalate and tartrate, with and without dyes, indicate that these salts are likewise efficacious in greatly increasing the corrosion resistance and producing a coloration which is relatively fast to light, heat and solvents.

The foregoing definitely indicates that a stannous salt solution alone is capable of greatly increasing the corrosion resistance of phosphate-coated ferrous metals and alloys, and that when used in conjunction with a compatible dye, it not only produces a further increase in corrosion

8 resistance, but also is capable of producing a distinctive coloration which is fast to light, heat, water and solvents. Moreover, the treatment does not produce appreciable dimensional changes in the article and the resultant coating is harder, i. e., more scratch-resistant, denser or more fine grained, and much more attractive than the untreated phosphate coating produced in accordance with conventional practices. A further advantageous feature of our treatment is that it may be carried out in a short time, e. g., a minute or two, and in a single operation. If desired, both the general appearance and corrosion resistance may be further enhanced by oiling, waxing or the like conventional treatment.

We claim:

1. The method of treating a metal article having an insoluble metal phosphate coating thereon produced by chemical reaction of the phosphate radical with the metal surface, which comprises subjecting said phosphate coating to the action of an aqueous solution of a stannous salt which is water soluble and water stable, the solution having an acidity insufficient to strip said phosphate coating, thereby to form an insoluble tin-metal-phosphate complex having a corrosion resistance greatly exceeding the original phosphate coating.

2. The method of treating a metal article having an insoluble metal phosphate coating thereon produced by chemical reaction of the phosphate radical with the metal surface, which comprises subjecting said phosphate coating to the action of an aqueous stannous chloride solution, the solution having an acidity insufficient to strip said phosphate coating, thereby to form an insoluble tin-metal-phosphate complex having a corrosion resistance greatly exceeding the original phosphate coating.

3. The method of treating metallic articles which comprises first forming a phosphate coating thereon by treatment with an aqueous solution containing a salt having the general formula  $M(H_2PO_4)_2$ , wherein M is a metal in the electro-motive series from manganese to iron, both inclusive and subsequently subjecting said phosphate coating to the action of an aqueous solution of a stannous salt which is water soluble and water stable, the solution having an acidity insufficient to strip said phosphate coating, and thereby to form an insoluble tin-metal-phosphate complex having a corrosion resistance greatly exceeding the original phosphate coating.

4. The method of treating metallic articles which comprises first forming a phosphate coating thereon by treatment with an aqueous solution containing a salt having the general formula  $M(H_2PO_4)_2$ , wherein M is a metal in the electro-motive series from manganese to iron, both inclusive and subsequently subjecting said phosphate coating to the action of an aqueous stannous chloride solution, the solution having an acidity insufficient to strip said phosphate coating, thereby to form an insoluble tin-metal-phosphate complex having a corrosion resistance greatly exceeding the original phosphate coating.

5. The method of treating a metal article having an insoluble metal phosphate coating thereon produced by chemical reaction of the phosphate radical with the metal surface, which comprises subjecting said phosphate coating to the action of an aqueous solution of a stannous salt which is water soluble and water stable, the solution having an acidity insufficient to strip said phosphate coating, and a dye compatible with

said stannous salt solution thereby to form an insoluble tin-metal-phosphate-dye complex having a corrosion resistance greatly exceeding the original phosphate coating and simultaneously imparting a coloration thereto.

6. The method of treating a metal article having an insoluble metal phosphate coating thereon produced by chemical reaction of the phosphate radical with the metal surface, which comprises subjecting said phosphate coating to the action of an aqueous stannous chloride solution and a dye compatible with said stannous chloride solution, the solution having an acidity insufficient to strip said phosphate coating, thereby to form an insoluble tin-metal-phosphate-dye complex having a corrosion resistance greatly exceeding the original phosphate coating and simultaneously imparting a coloration thereto.

7. The method of treating a metal article having an insoluble metal phosphate coating thereon produced by chemical reaction of the phosphate radical with the metal surface, which comprises subjecting said phosphate coating to the action of an aqueous treating solution containing from 2% to 25% of a stannous salt which is water soluble and water stable, the solution having an acidity insufficient to strip said phosphate coating, thereby to form an insoluble tin-metal-phosphate complex having a corrosion resistance greatly exceeding the original phosphate coating.

8. The method of treating a metal article having an insoluble metal phosphate coating thereon produced by chemical reaction of the phosphate radical with the metal surface, which comprises subjecting said phosphate coating to the action of an aqueous treating solution containing from 2% to 25% of a stannous chloride, the solution having an acidity insufficient to strip said phosphate coating, thereby to form an insoluble tin-metal-phosphate complex having a corrosion resistance greatly exceeding the original phosphate coating.

9. The method of treating metallic articles which comprises first forming a phosphate coating thereon by treatment with an aqueous solution containing a salt having the general formula  $M(H_2PO_4)_2$ , wherein M is a metal in the electro-motive series from manganese to iron, both inclusive and subsequently subjecting said phosphate coating to the action of an aqueous treating solution containing from 2% to 25% of a stannous salt which is water soluble and water stable, the solution having an acidity insufficient to strip said phosphate coating, thereby to form an insoluble tin-metal-phosphate complex having a corrosion resistance greatly exceeding the original phosphate coating.

10. The method of treating metallic articles which comprises first forming a phosphate coating thereon by treatment with an aqueous solution containing a salt having the general formula  $M(H_2PO_4)_2$ , wherein M is a metal in the electro-motive series from manganese to iron, both inclusive and subsequently subjecting said phosphate coating to the action of a treating solution containing 2% to 25% stannous chloride, the solution having an acidity insufficient to strip said phosphate coating, thereby to form an insoluble tin-metal-phosphate complex having a corrosion resistance greatly exceeding the original phosphate coating.

11. The method of treating a metal article having an insoluble metal phosphate coating thereon

produced by chemical reaction of the phosphate radical with the metal surface, which comprises subjecting said phosphate coating to the action of an aqueous treating solution containing from 2% to 25% of a stannous salt which is water soluble and water stable, the solution having an acidity insufficient to strip said phosphate coating, and from 0.1% to 10% (based on the weight of the treating solution) of a dye compatible with said stannous salt solution, thereby to form an insoluble tin-metal-phosphate-dye complex having a corrosion resistance greatly exceeding the original phosphate coating.

12. The method of treating a metal article having an insoluble metal phosphate coating thereon produced by chemical reaction of the phosphate radical with the metal surface, which comprises subjecting said phosphate coating to the action of an aqueous treating solution containing from 2% to 25% of stannous chloride and from 0.1% to 10% (based on the weight of the treating solution) of a dye compatible with said stannous chloride solution, the said stannous chloride solution having an acidity insufficient to strip said phosphate coating thereby to form an insoluble tin-metal-phosphate-dye complex having a corrosion resistance greatly exceeding the original phosphate coating.

13. An article having a protective coating consisting essentially of an insoluble tin-metal-phosphate complex produced in accordance with the process of claim 1.

14. An article having a protective coating consisting essentially of an insoluble tin-metal-phosphate complex produced in accordance with the process of claim 3.

15. An article having a protective coating consisting essentially of an insoluble tin-metal-phosphate-dye complex produced in accordance with the process of claim 5.

16. An article having a protective coating consisting essentially of an insoluble tin-metal-phosphate complex produced in accordance with the process of claim 9.

BERTHA S. TUTTLE.  
THADDEUS NAVOY.

#### REFERENCES CITED

The following references are of record in the file of this patent:

#### UNITED STATES PATENTS

| Number       | Name          | Date          |
|--------------|---------------|---------------|
| 1,303,627    | Baines        | May 13, 1919  |
| 55 1,329,573 | Allen         | Feb. 3, 1920  |
| 1,426,675    | Schlotter     | Aug. 22, 1922 |
| 1,466,126    | Fink          | Aug. 28, 1923 |
| 1,514,494    | Williams      | Nov. 4, 1924  |
| 1,694,820    | Harris        | Dec. 11, 1928 |
| 60 2,200,615 | Boyle         | May 14, 1940  |
| 2,236,549    | Darsey et al. | Apr. 1, 1941  |
| 2,295,063    | Tuttle        | Sept. 8, 1942 |
| 2,304,299    | Boyle et al.  | Dec. 8, 1942  |
| 2,314,565    | Thompson      | Mar. 23, 1943 |

#### FOREIGN PATENTS

| Number  | Country | Date         |
|---------|---------|--------------|
| 731,994 | France  | June 6, 1932 |

#### OTHER REFERENCES

70 Cox: "Hair Dyes. I. The chemistry and analysis of henna," The Analyst (England), vol. 63 (1938), pages 397-404.